# EUROPEAN PATENT SPECIFICATION

(11) **EP 0 148 821 B1**
(45) Date of publication and mention of the grant of the patent: **13.07.1988**
(21) Application number: 83902467.6
(22) Date of filing: 27.05.1983
(51) Int. Cl.: B22F 3/00, C22C 29/00

(54) **METHOD OF MAKING AND USING A TITANIUM DIBORIDE COMPRISING BODY**
VERFAHREN ZUR HERSTELLUNG UND VERWENDUNG EINES TITANDIBORID ENTHALTENDEN KÖRPERS
PROCEDE DE FABRICATION ET D'UTILISATION D'UN CORPS COMPORTANT DU DIBORURE DE TITANE

(43) Date of publication of application: 24.07.1985
(73) Proprietor: FORD MOTOR COMPANY LIMITED, Brentwood, Essex CM13 3BW (GB); FORD-WERKE AKTIENGESELLSCHAFT, 50725 Köln (DE); FORD FRANCE SOCIETE ANONYME, 92506 Rueil Malmaison Cedex (FR)
(72) Inventor: MOSKOWITZ, David, Southfield, MI 48076 (US); PHILLIPS, Charles, W., Ann Arbor, MI 48104 (US)
(74) Representative: Messulam, Alec Moses
(86) International application number: US8300843
(87) International publication number: WO8404713

(56) References cited:
- GB-A- 392 038
- GB-A- 866 119
- JP-A-75 151 911
- JP-A-80 154 544
- SU-A- 514 031
- SU-A- 523 954
- SU-A- 824 677
- US-A- 2 116 400
- US-A- 2 799 912
- US-A- 3 052 538
- US-A- 3 313 605
- US-A- 4 145 213

## Description

This invention relates to the art of making heat fused titanium boride bodies useful as cutting tools, particularly for aluminum based materials.

Considerable interest, as a potential tool material, has been aroused in the use of abrasion resistant materials which consist of or contain boron, usually in the form of a boride of titanium. The material is usually fabricated by cementing together the titanium boride material with a metallic binder which may include iron, nickel, or cobalt. However, utilizing such metal binders has not met with success because of (a) unsatisfactory strength and hardness at high temperatures, and (b) the processing temperature required for formation of the bond between the particles is too high (see U.S. Patent 3,256,072).

To create a higher density sintered body with higher mechanical strength, the art has attempted to replace such metal binders with a combinaton of two separate components, the first of which includes a nickel phosphide or nickel phosphorus alloy, and the second consists of a metal selected from the group comprising chromium, molybdenum, rhenium, and the like, or a metal diboride, chromium diboride, or zirconium diboride (see U.S. Patent 4,246,027). However, this particular replacement and chemistry has not proved entirely successful because the resulting combination of hardness and strength still remains below desired levels and still requires expensive hot pressing to achieve densification. But, more importantly, the presence of phosphorus in this prior art material can make the material unsuitable for machining aluminium based materials due to embrittlement.

SU-A-514031 discloses a sintered titanium diboride material for cutting tools, consisting of 63.4% TiB₂, 13% Co and 23.1% WC.

GB-392038 discloses a sintered hard alloy consisting of 75% titanium boride 20% titanium carbide and 5% nickel.

According to the invention, there is provided a method of making a high titanium diboride comprising body, useful when shaped as a cutting tool, by the steps comprising compacting a powder mixture including an iron group metal and titanium diboride and sintering said compact to form said body, characterised in that said mixture includes 5-20% by weight of iron group metal selected from the group consisting of iron, nickel and cobalt, or an alloy thereof, 0-10% by weight of titanium carbide, 0.2-1% oxygen, 4% or less than 4% graphite and the remainder being titanium diboride, said mixture being milled prior to compacting to a maximum particle size of 5 11m and said compact being heated to a temperature sufficient to densify said compact to at least 97% of full theoretical density, the graphite being present in the mixture prior to sintering in order to reduce the oxygen content in the sintered body, the mixture losing up to 2% by weight of graphite by reaction with the oxygen during sintering.

Further according to the invention, there is provided a titanium diboride comprising body which is a heat fused product of a compacted mixture including an iron group metal and titanium diboride, characterised in that said mixture includes 5-20% by weight of an iron group metal selected from the group consisting of cobalt, nickel, and iron, or an alloy thereof, 0-10% by weight of titanium carbide, 0.2-1% oxygen, 4% or less than 4% graphite, and the remainder being titainium diboride, said body exhibiting a hardness of at least 90 Rockwell A and a transverse rupture strength of at least 6.89x10⁵ kPa (100,000 psi), said heat fused product having grain size equal to or less than 5 11m and exhibiting a loss of up to 2% by weight of graphite during the sintering of the compacted mixture.

Preferably, the metal binder consists of an alloy of iron and nickel with the nickel occupying 20-50% of the alloy. Alternatively, the binder may consist of an alloy comprising iron, nickel, and cobalt with nickel occupying 5-10% of the alloy and cobalt constituting 2.5-5% of the alloy.

The method of using titanium diboride comprising body of the present invention essentially comprises relatively moving a titanium diboride based cutting tool against the aluminum based material to machine cut said material at a relative surface speed of at least 120 m per minute (400 surface feet per minute) and depth of cut of from 0.0254_{^}0.635 cms (0.010-.250 inch).

It will be shown that composite materials produced from titanium diboride powder combined with either iron, nickel, cobalt, or alloys of such metals, and when prepared in a manner that the titanium diboride particle size in the final sintered product is less than 5 µm, will produce a combination of physical characteristics of hardness, strength, and density superior to titanium diboride based articles prepared by prior art techniques.

A preferred method for fabricating the material of this invention is as follows.

### 1. Mixing.

A powder mixture of 5-20% by weight of a metal binder, the metal elements being selected from the iron group (here defined to be the group consisting of cobalt, nickel and iron), and the remainder of said mixture being essentially titanium diboride, except for 0.2 to 1.0% oxygen and up to 4% graphite. The titanium diboride powder has a purity of 99% or greater, and has typical contaminants which comprise 0₂, N₂ and Fe. The metal binder powder has a purity of 99.5% or greater. For purposes of the preferred embodiment, 90 parts by weight of a titanium diboride powder was mixed with 10 parts by weight of electrolytic iron powder. Four parts by weight of carbowax 600 (a polyethylene glycol) was stirred into the mixture to form a powder slurry.

A 200 gram batch of these constituents was ball milled under acetone for 72 hours in a stainless steel mill having a chamber approximately 12 centimeters in diameter and 12 centimeters long. Milling media in the form of 1300 grams of TiC based media, approximately 1 centimeter in diameter and 1 centimeter long, was employed. The acetone was then evaporated and the dried powder mix was screened to provide a powder mixture having a maximum particle size of 5 pm.

### 2. Compacting

Specimen bodies of the powder mixture were compacted at a pressure of 69-207 MPa (5-15 tons per square inch), preferably 138 MPa (10 tons per square inch), and then heated to a temperature of about 673°C for one hour in a dry hydrogen atmosphere to dewax or remove the Carbowax 600 from the mixture.

### 3. Heating to full densification

The compacted bodies then were sintered by heating each in a furnace which was evacuated to a pressure of 0.4 Pa (0.3 microns of mercury) and heated to a temperature of about 1540°C. The bodies were held at the sintering temperature for a period of about 15 minutes. Titanium carbide crystalline grains were used as the inert substrate material. The resulting sintered product possessed a hardness of 94 Rockwell A, an average transverse rupture strength of 7.92xlO^{s} kPa (115,000 psi), and a density over 97% of the theoretical apparent density.

It was found during experimentation with this process that the presence of a certain amount of oxygen, either as an oxide or as an elemental amount in the mixture, caused the hardness and transverse rupture strength to be less than desired. It was found that the addition of up to 4% graphite (free carbon) to the mixture, prior to milling, removed the influence of the high oxygen content and restored the physical parameters to that of specimens which did not have such oxygen content.

Iron, cobalt, and nickel, as well as their alloys, have proved to be successful binders for titanium diboride. As long as the titanium diboride grain size in the final sintered compact is maintained equal to or below 5 pm, good properties have been obtained using any of the iron group metals or their alloys as a binding agent.

### Examples

Several samples were prepared according to the preferred mode wherein a specific powder mixture was prepared with titanium diboride as the base material and a metal binder in varying amounts of the selected elements. Some samples employed titanium carbide as a replacement for titanium diboride, and others contained an addition of graphite. The results from processing such mixtures according to the preferred method are illustrated in Table I, which sets forth the specific hardness, transverse rupture strength, and density for each of the specimens as processed. A hardness of no less than 90 Rockwell A and a transverse rupture strength of no less than 6.89x10⁵ kPa (100,000 psi) is considered satisfactory.

The latter samples 7 and 8 in Table I draw a comparison between equal mixtures of titanium diboride, titanium carbide, and nickel, one sample producing a lower hardness and strength than the other sample; the difference between the two mixtures is the oxygen content (sample 7 having 0.19% O2 and sample 8 having 0.95% O2), When up to 2% by weight of the composition consisted of graphite, the hardness and strength of sample 8 were restored to the level of that of a mixture having a lower level of oxygen (see sample 9). The beneficial effect of graphite additions to compositions having a higher oxygen content is important. Chemical analysis for carbon content of sintered specimens with various carbon additions up to 4% by weight indicate losses of carbon during sintering up to a maximum loss of about 2% by weight. It would appear then that the beneficial effect of carbon additions to compositions prepared is due to the reduction of oxygen that is present as an oxide or oxides in the titanium diboride powder.

Titanium diboride compacts produced in the manner described above have been found particularly suitable for use in an unobvious manner for the machining of aluminum and aluminum alloys. It has been found that titanium diboride is nonreactive in the presence of molten aluminum; and when used as a cutting tool against aluminum based materials, the titanium diboride based cutting tool exhibits a low affinity for aluminum based workpieces, provided the strength and hardness of the cutting material exceeds 6.89x10⁵ kPa (100,000 psi) and 90 Rockwell A, respectively. The machining test results displayed in Table II demonstrate the unobvious utility of the use of this material for machining aluminum based materials. Cutting tests were run both with and without coolants to compare the titanium diboride based cutting tool material with commercial grade C-3 tungsten carbide based cutting tools. The machining workpiece was continuously cast aluminum alloy AA 333 (8.5% silicon, 3.6% copper, and .4% magnesium). The workpieces were used both in the unmodified and sodium modified conditions. The tool was comprised of a material processed according to the preferred mode and having 90% TiB₂ and 10% Ni. The tool configuration was SPG 422. The conditions of machine cutting were 0.28 cm (.011 inches) per revolution and depth of cut .15 cms (.060 inch). The cutting fluid was 5% soluble oil in water.

The average tool life is given in the Table in minutes; the life is measured up to a condition when the tool experiences .025 cms (.010 inch) of flank wear. The average tool life for the titanium diboride based tool was 2.36 times greater than that of the commercial tungsten carbide based tool for the unmodified aluminum. A similar improvement in tool life occurred with respect to the use of the titanium diboride tool on sodium modified aluminum; the improvement in tool life was 2.52 times the life of the tungsten carbide tool. It is worth noting that, at 2000 surface feet per minute, this improvement took place when machining dry as well as when coolant was present.

### Composition

The resulting material from the practice of the preferred mode is unique because it consists of a titanium diboride based material including 5-20% by weight of an iron group metal binder, said binder being selected from the group consisting of cobalt, nickel and iron, or alloys thereof 0 to 10 wt.% titanium carbide, and the remainder being titanium diboride except for 0.2 to 1.0% oxygen and up to 2% graphite, said material being the heat fused product of said compacted mixture and exhibiting a hardness of at least 90 Rockwell A and a transverse rupture strength of at least 6.89x10⁵ kPa (100,000 psi), said heat fused product having a titanium diboride grain size equal to or less than 5 pm.

## Claims

1. A method of making a high titanium diboride comprising body, useful when shaped as a cutting tool by the steps comprising compacting a powder mixture including an iron group metal and titanium diboride and sintering said compact to form said body, characterised in that said mixture includes 5-20% by weight of iron group metal selected from the group consisting of iron, nickel and cobalt, or an alloy thereof, 0-10% by weight of titanium carbide, 0.2-1% oxygen, 4% or less than 4% graphite and the remainder being titanium diboride, said mixture being milled prior to compacting to a maximum particle size of 5 11m and said compact being heated to a temperature sufficient to densify said compact to at least 97% of full theoretical density, the graphite being present in the mixture prior to sintering in order to reduce the oxygen content in the sintered body, the mixture losing up to 2% by weight of graphite by reaction with the oxygen during sintering.

2. A method as claimed in Claim 1, in which said mixture includes an alloy said mixture includes an alloy of iron and nickel, said nickel occupying 20-50% by weight of said alloy.

3. A method as claimed in Claim 1, in which said mixture includes an alloy of iron, nickel, and cobalt wherein said cobalt constitutes 2.5-5% by weight of said alloy and said nickel being 5-10% by weight of said alloy.

4. A method as claimed in any one of Claims 1 to 3, in which said sintering is carried out in an evacuated furnace to a pressure of under 2.66 Pa (20 microns of mercury) and heated to a temperature of 1500-1570°C for a period of 10-30 minutes.

5. A titanium diboride comprising body which is a heat fused product of a compacted mixture including an iron group metal and titanium diboride, characterised in that said mixture includes 5-20% by weight of an iron group metal selected from the group consisting of cobalt, nickel, and iron, or an alloy thereof, 0-10% by weight of titanium carbide, 0.2-1% oxygen, 4% or less than 4% graphite, the remainder being titanium diboride, said body exhibiting a hardness of at least 90 Rockwell A and a transverse rupture strength of at least 6.89x10⁵ kPa (100,000 psi), said heat fused product having grain size equal to or less than 5 µm and exhibiting a loss of up to 2% by weight of graphite during the sintering of the compacted mixture.

## Patentansprüche

1. Verfahren zur Herstellung eines hoch Titandiboridhaltigen Körpers, welchen man in Form eines Schneidewerkzeugs benützen kann, durch schrittweise Pressung einer Pulvermischung, die ein Ferrometall und Titandiborid enthält, und Sinterung dieses Presslings zur Bildung jenes Körpers, dadurch gekennzeichnet, daß sich besagte Mischung aus 5-20 Gew.-% aus der Gruppe Eisen, Nickel und Kobalt oder einer Legierung davon ausgewählten Ferrometalls, aus 0-10 Gew.-% Titancarbid, aus 0,2-1 % Sauerstoff, aus 4% oder weniger als 4% Graphit und als Rest aus Titandiborid zusammensetzt, wobei man die Mischung vor dem Pressen auf eine Teilchengröße von maximal 5 um mahlt und diesen Pressling auf eine zu seiner Verdichtung auf wenigstens 97% der vollen theoretischen Dichteerwartung ausreichenden Temperatur erhitzt und wobei Graphit vor dem Sintern in der Mischung gegenwärtig ist, um den Sauerstoffgehalt im gesinterten Körper herabzusetzen und die Mischung bis zu 2 Gew.-% Graphit durch Reaktion mit Sauerstoff während des Sinterns verliert.

2. Verfahren nach Anspruch 1, worin besagte Mischung eine Legierung aus Eisen und Nickel enthält, wobei das Nickel 20-50 Gew.-% dieser Legierung einnimmt.

3. Verfahren nach Anspruch 1, worin besagte Mischung eine Legierung aus Eisen, Nickel und Kobalt enthält, wobei das Kobalt 2.5-5 Gew.-% dieser Legierung und das Nickel 5--10 Gew.-% dieser Legierung ausmacht.

4. Verfahren nach einem der Ansprüche 1 bis 3, worin jene Sinterung in einem auf einen Druck unter 2,66 Pa (20 Mikron Quecksilber) evakuierten Brennofen und unter 10-30 Minuten andauernder Erhitzung auf eine Temperatur von 1500-1570°C vorgenommen wird.

5. Titandiboridhaltiger Körper als hitzerverschmolzenes Produkt einer gepressten, ein Ferrometall- und Titandiborid enthaltenden Mischung, dadurch gekennzeichnet, daß sich besagte Mischung aus 5-20 Gew.-% aus der Gruppe Eisen, Nickel und Kobalt oder einer Legierung davon ausgewählten Ferrometalls, aus 0-10 Gew.-% Titancarbid, aus 0,2-1 % Sauerstoff, aus 4% oder weniger als 4% Graphit und als Rest aus Titanborid zusammensetzt, wobei jeder Körper wenigstens eine Härte 90 nach Rockwell A und eine Biegebruchfestigkeit von wenigstens 6,89 · 10⁵ kPa (100.000 psi) und das hitzeverschmolzene Produkt eine Teilchengröße von gleich oder weniger als 5 um bei bis zu 2 Gew.-% Graphitverlust während des Sinterns der gepressten Mischung aufweist.

## Revendications

1. Procédé de fabrication d'un corps comprenant une haute teneur en diborure de titane, utile comme outil de coupe après façonnage, selon les stades comprenant la compression d'un mélange en poudre comprenant un métal du group du fer et un diborure de titane, et le frittage dudit produit comprimé pour former ledit corps, caractérisé en ce que ledit mélange comprend de 5 à 20% en poids d'un métal du groupe du fer choisi parmi le fer, le nickel et le cobalt ou un de leurs alliages, de 0 à 10% en poids de carbure de titane, de 0,2 à 1 % d'oxygène, 4% ou moins de 4% de graphite, le reste étant du diborure de titane, ledit mélange étant broyé avant la compression à une taille maximale des particules de 5 µm, et ledit produit comprimé étant chauffé à une température suffisante pour densifier celui-ci jusqu'à au moins 97% de la masse volumique théorique maximale, le graphite étant présent dans le mélange avant le frittage afin de réduire la teneur en oxygène dans le corps fritté, le mélange perdant jusqu'à 2% en poids de graphite par réaction avec l'oxygène pendant le frittage.

2. Procédé selon la revendication 1, dans lequel ledit mélange comprend un alliage de fer et de nickel, le nickel représentant de 20 à 50% du poids dudit alliage.

3. Procédé selon la revendication 1, dans lequel ledit mélange comprend un alliage de fer, de nickel et de cobalt, le cobalt représentant de 2,5 à 5% en poids dudit alliage, et le nickel représentant de 5 à 10% en poids dudit alliage.

4. Procédé selon l'une quelconque des revendications 1 à 3, dans lequel ledit frittage est effectué dans un four dont on a réduit la pression jusqu'à moins de 2,66 Pa et chauffé à une température de 1 500 à 1 570°C pendant une période de 10 à 30 minutes.

5. Corps comprenant du diborure de titane, qui est un produit fusionné à chaud d'un mélange comprimé comprenant un métal du groupe du fer et du diborure de titane, caractérisé en ce que ledit mélange comprend de 5 à 20% en poids d'un métal du groupe de fer choisi parmi le cobalt, le nickel et le fer ou un de leurs alliages, de 0 à 10% en poids de carbure de titane, de 0,2 à 1% d'oxygène, 4% ou moins de 4% de graphite, le reste étant du diborure de titane, ledit corps présentant une dureté Rockwell A d'au moins 90 et une résistance à la rupture transversale d'au moins 6,89x10⁵ kPa, ledit produit fusionné à chaud ayant une taille des grains égale ou inférieure à 5 pm et présentant une perte de graphite atteignant 2% en poids pendant le frittage du mélange comprimé.
